

A. B. WARING.  
METHOD OF MAKING FELT HATS.  
APPLICATION FILED NOV. 19, 1912.

1,115,354.

Patented Oct. 27, 1914.

Fig. 1,



Fig. 2,



Fig. 3,



WITNESSES  
J. D. Barbour  
F. Graves

INVENTOR  
Arthur B. Waring  
BY  
E. W. Marshall  
ATTORNEY

# UNITED STATES PATENT OFFICE.

ARTHUR B. WARING, OF NEW YORK, N. Y.

## METHOD OF MAKING FELT HATS.

1,115,354.

Specification of Letters Patent. Patented Oct. 27, 1914.

Application filed November 19, 1912. Serial No. 732,202.

*To all whom it may concern:*

Be it known that I, ARTHUR B. WARING, a citizen of the United States of America, and a resident of New York, county and 5 State of New York, have invented certain new and useful Improvements in Methods of Making Felt Hats, of which the following is a specification, reference being had to the accompanying drawing, forming a part 10 thereof.

My invention relates to a novel process of treating and making hats and to the hats treated or made according to this improved process.

15 The invention relates more specifically to felt hats, and its object is to provide a simple method for making hats of this particular type, of novel and pleasing appearance.

I will now describe my invention in the 20 following specification and then point out the novel features thereof in appended claims.

Referring to the drawings: Figure 1 is a perspective view of a hat made according to 25 the present invention. Fig. 2 is a side elevation of a block upon which such a hat as that shown in Fig. 1 may be treated. Fig. 3 is an elevation of a pattern plate or form which may be used in carrying out 30 in a slightly different manner the herein described process. In this figure a part of the pattern plate is broken away to more clearly show its construction.

Like characters of reference designate 35 corresponding parts in all the figures.

A felt hat of usual form is shown in Fig. 1 at 10. Upon both the crown and the rim of this hat appears a design or pattern which may be produced in the novel manner 40 which I have invented. This design effect is produced by abrading or rubbing with sand paper or other suitable material certain portions of the surface of the hat body to effect a contrast in appearance between the abraded 45 and other portions of the body. In Fig. 1 the abraded portions are designated by 11 and the other portions by 12.

A satisfactory manner of accomplishing the desired results is as follows:—a hat 50 body is formed of animal fiber,—fur or wool—with some other kind or kinds of fiber mixed with it, for example, about fifteen per cent. of a vegetable fiber, such as ramie may be used, although obviously I do not 55 limit myself to any specific proportions or

to this particular material. The body is then shrunk in the usual manner. This causes the animal fibers to become felted together, but as the ramie has no felting properties it works into the body of the 60 material and becomes covered by the fur or wool. The hat is then immersed in a dye for animal fibers which does not have a like effect upon the vegetable fibers. A satisfactory jet black dye for the fur has practically no effect upon the ramie which retains its original whiteness. If desired, the ramie may be colored before it is mixed with the fur, but as dyeing injures the felting 65 property of either fur or wool, it is better to do the dyeing of the animal fiber after the shrinking process. If preferred the ramie may be dyed and the animal fiber left in its natural color, or animal and vegetable fibers of different colors used and both left in their 70 natural colors. A hat made as thus described has substantially the same appearance as one made of animal fiber alone and it may be pounced or abraded a sufficient amount to reduce it to a smooth surface without materially affecting its appearance. I have however, discovered that when certain portions of such a hat are abraded more than other portions, the animal fibers which cover the ramie may be removed, thus materially 75 changing the appearance of such abraded portions. That is, if the animal fiber is dyed black the abraded portions may uncover the ramie a sufficient amount to make such portions gray, or if further abraded such portions may have a decidedly white 80 appearance, if the ramie is uncolored, or red or green, or any other color which may have been given to the ramie.

It is the object of the present invention to 85 utilize this discovery in producing in felt hats, designs of any desired pattern. A simple manner of accomplishing this result is to provide a block 13 such as that shown in Fig. 2 with alternately raised and depressed portions over its surface. The particular block shown in the drawings is made to produce upon a hat the design illustrated in Fig. 1. To this end it is constructed with raised horizontal ribs 14 and transverse ribs 15 with intermediate depressed portions 16 between the ribs. The hat may be placed over such a block and pressed or forced onto it. This causes portions of the fabric which are between the raised ribs to be pressed in 110

away from the general contour of the body, thus embossing the design of the block in the body of the hat. While on such a block the pouncing or abrading may be done, 5 preferably with a coarser sand paper than that used for the surfacing abrasion. The raised portions of the fabric will then be acted upon sufficiently to remove the felted covering of the vegetable fibers and to have 10 a combing effect upon the fibers without the depressed portions being materially affected. This will result in the production of the desired design or pattern. After this the embossing is pressed out. It is to be understood 15 that the rim of the hat may be similarly treated.

Of course instead of raised ribs on the block these portions may be depressions or grooves and the intermediate portions 20 raised. Such a block would reverse the pattern produced on the hat.

The pattern plate or form shown in Fig. 3 is a shell 17 of sheet metal through which slits or openings 18 are cut of such shape and 25 size and relative positions as to form a desired pattern. The hat body is to be placed inside of this shell and forced into it by means of a rigid block or by an expandable bulb or bag. This will bring the outer surface 30 of the hat up against the inner surface of the shell or may even cause some of the fabric to protrude through the slits or openings in the shell. Such portions of the hat as are opposite the slits may be abraded as 35 before described.

It is well within my invention to treat fabrics with local abrasion other than those composed of unlike fibers for the production thereon of designs. It is for example, feasible 40 to treat a surface-dyed fabric in which a design has been embossed as herein described, to obtain pleasing effects. Of course the process is not necessarily limited to the treatment or manufacture of hats. It is also 45 possible to apply local abrasion to the surface of a fabric without previously embossing the fabric or without protecting the portions which are not to be abraded by a shell. That is, a desired design may be produced upon 50 the fabric by localizing the abrasion by hand. I have described several ways in which my process may be used to show that I do not limit myself to any specific mechanism or manner of using it. By the use of 55 this invention felt hats may be made which closely simulate hats made of woven fabric with designs in colors woven in them. The product of this process is, I believe, new with me and I wish to cover it as well as the 60 process.

What I claim is:

1. The process of producing a designed fabric consisting in making the fabric with the inner portion thereof containing a material 65 unlike that on its surface, embossing a

design on the surface and abrading the embossed portions to disclose the inner unlike material.

2. The process of treating felt containing a percentage of non-felting material that 70 consists in abrading the felt surface in predetermined portions to disclose the non-felting material in the form of a design.

3. The process of producing a designed fabric that consists in felting a mixture containing a large percentage of animal fiber 75 and a small percentage of vegetable fiber, treating the fabric with a dye which acts more upon the animal fiber than upon the vegetable fiber, and locally abrading the surface of the fabric to disclose the vegetable fiber in the form of a design. 80

4. The process of making felt which comprises mixing a large percentage of animal fiber and a small percentage of vegetable 85 fiber of a predetermined appearance, shrinking the mixture to cause the animal fiber to cover the vegetable fiber, dyeing the animal fiber, and in locally abrading the surface of the felt thus formed to disclose the vegetable 90 fiber in the form of a design.

5. The process of producing hats comprising making a hat body of intermingled fibers of unlike materials, felting said body thereby covering the fibers of one of the materials, 95 and in locally abrading portions of the surface of the body to uncover in the abraded portions the covered fibers.

6. The process of producing felt hats with designs in their fabrics that consists in felting a mixture containing a predetermined percentage of a non-felting material, embossing a design thereon, and abrading the raised portions to disclose the non-felting material. 100

7. The process of producing hats comprising making a hat body of intermingled fibers of unlike materials differently affected by dye, felting said body thereby covering the fibers of one of the materials, dyeing the 110 body, and locally abrading portions of the surface of the body to uncover in the abraded portions the covered fibers.

8. The process of producing hats comprising making a hat body of intermingled fibers of animal fiber and vegetable fiber, shrinking said body thereby causing the animal fiber to felt and to cover the vegetable fiber, dyeing the body with a material which affects the animal fiber differently than it does 120 the vegetable fiber, and locally abrading portions of the surface of the body to uncover in the abraded portions the covered fibers.

9. The process of producing felt hats that consists in felting in the form of a hat body 125 a mixture containing a small percentage of non-felting material whereby said non-felting material is covered in the fabric, embossing a design in said fabric and abrading the surface to disclose the non-felting material. 130

10. The process of producing hats comprising making a hat body of intermingled fibers of animal fiber and vegetable fiber, shrinking said body thereby causing the animal fiber to felt and to cover the vegetable fiber, dyeing the body with a material which affects the animal fiber differently than it does the vegetable fiber, embossing a design in the body and then subjecting said body to abrasion.

11. The process of producing a designed fabric consisting in making the fabric with the inner portion thereof containing a mate-

rial unlike that on its surface, embossing a design of the surface and abrading the embossed portions to disclose the inner unlike material, and then pressing out the embossing.

In witness whereof I have hereunto set my hand this 16th day of November, in the presence of two subscribing witnesses.

ARTHUR B. WARING.

Witnesses:

ERNEST W. MARSHALL,  
JULIUS TACKMAN.